

## 1

3,091,552

### PROCESS FOR INCREASING THE RESISTANCE OF POLYACRYLONITRILE FIBERS TO DISCOLORATION

Vera Isabella Furness, Coventry, England, and Hector Douglas Mackenzie, Mhlambanyati, near Mbabane, Swaziland, assignors to Courtaulds Limited, London, England, a British company

No Drawing. Filed Apr. 28, 1961, Ser. No. 106,181  
Claims priority, application Great Britain May 6, 1960  
4 Claims. (Cl. 117—138.8)

This invention concerns the treating of artificial fibres of polyacrylonitrile to render them more stable to discolouration. In the word "fibres" we include continuous filaments as well as staple fibre. By "polyacrylonitrile" we mean homopolymers of acrylonitrile and copolymers containing at least 80 percent by weight of acrylonitrile.

Polyacrylonitrile fibres exhibit a tendency to discolour which may display itself when the fibres are subjected to heating, for example during drying or hot-stretching of the fibres, or during steaming. Various suggestions have been made for modifying the polyacrylonitrile solution which is spun to form the fibres, in order to improve the colour of the freshly-spun fibres. However, it is desirable that a treatment be made available, which can be applied to the fibres after spinning, for improving the colour stability of spun fibres of poor stability. It is an object of this invention to provide such a treatment.

According to this invention, a process for treating artificial fibres of polyacrylonitrile to render them more resistant to heat-discoloration and/or steam discolouration comprises applying to the surface of the fibres, before they have been first dried, an aqueous solution or suspension of a reducing agent which does not have any adverse effect on the fibres. Typical reducing agents which may be used are thiourea dioxide (also known as formamidine sulphinic acid), sodium and potassium metabisulphite, formaldehyde and addition compounds of formaldehyde with compounds which do not themselves adversely affect the fibres. The formaldehyde addition compounds which may be used include that with sodium bisulphite, while sodium formaldehyde sulphoxylate is unsuitable because of the deleterious effect of the second component. Formaldehyde may also be used in the form of its polymer paraformaldehyde.

The application of the solution or suspension of reducing agent to the fibres may advantageously be carried out by passing a continuously-moving bundle of filaments through a bath of the agent at a stage in the fibre production-line which precedes the drier. If desired, the treatment according to this invention may be combined with other treatments such as the application of a finish to the fibres.

The solution or suspension of reducing agent may contain between 0.1 percent and 10 percent of reducing agent by weight, preferably less than 5 percent. Solutions containing of the order of 0.5 to 2 percent of reducing agent by weight have proved particularly useful.

The treatment according to this invention may be carried out using a solution or suspension which is at room temperature or at an elevated temperature. If the treatment is combined with any other treatment of the fibres which makes elevated temperatures necessary or desirable, such temperatures may be used without objection.

The invention will now be further described by means of the following examples, in which percentages are by weight unless stated otherwise:

#### Example 1

Undried polyacrylonitrile filaments spun from a solution in sodium thiocyanate solution were immersed for

## 2

2 seconds at 20° C. in a solution of sodium formaldehyde bisulphite prepared from 6 g. of a 40 percent solution of formaldehyde, 6 g. of sodium metabisulphite and 350 cc. of water. They were then dried at 80° C.

Treated and untreated fibres were compared (a) after steaming for half an hour under a steam pressure of 20 p.s.i. and (b) after heating in air at 150° C. for 30 minutes. In each case the treated fibre showed less discolouration than the untreated fibre, to an extent readily detectable by the unaided eye.

In the remaining examples, the fibre colour where given has been determined as fibre yellowness (Y) from the equation

$$Y = \frac{R - B}{G}$$

where R, B and G are the reflectance ratios in red, blue and green respectively, as measured on a "Colormaster" differential colorimeter.

#### Example 2

Undried polyacrylonitrile filaments were immersed in an aqueous bath containing 1 percent of a soft finish agent well-known in the art and 2 percent of sodium formaldehyde bisulphite. The treated fibres, after drying at 80° C. had a fibre colour of 0.093, which was increased only to 0.095 by steaming for a total of 12 minutes under a steam pressure of 10 p.s.i.

Similar fibres treated in a bath containing the soft finish agent alone showed a fibre colour after steaming of 0.120.

#### Example 3

Undried polyacrylonitrile filaments were treated by immersion for 5 seconds in a bath consisting of 5 g. of paraformaldehyde suspended in 100 cc. of water. The fibres were then dried at 80° C.

After steaming for half an hour at 20 p.s.i. the treated fibres showed a colour of 0.082, compared with 0.180 for steamed untreated fibres.

#### Example 4

Undried polyacrylonitrile filaments were immersed for 30 seconds at room temperature in filtered aqueous solutions of thiourea dioxide at pH 5.4, after which excess liquor was squeezed out by rollers and the fibres were dried for 2 hours at 80° C. Untreated fibres and fibres treated in solutions of varying concentration were subjected either to heating at 130° C. for 30 minutes or to steaming for 30 minutes at 10 p.s.i. The following table gives the fibre colour of the various samples:

| Treatment Bath   | Colour after drying | Colour after heating at 130° C. | Colour after steaming |
|------------------|---------------------|---------------------------------|-----------------------|
|                  |                     |                                 | 55                    |
| Untreated.....   | 0.094               | 0.250                           | 0.150                 |
| 1% solution..... | 0.101               | .....                           | 0.104                 |
| 2% solution..... | 0.097               | 0.126                           | 0.107                 |
| 5% solution..... | 0.083               | .....                           | 0.106                 |

It will be seen from the foregoing Examples 1 to 4 that treatment according to the invention has the effect of improving the colour of the fibres after heating to higher temperatures or steaming, and in some cases improves the fibre colour of the dried fibre.

65 What we claim is:

1. A process for increasing the resistance of polyacrylonitrile fibres to discolouration, comprising applying to the never-dried fibres in an aqueous medium a reducing agent which has no adverse effect on the fibre.

2. A process for increasing the resistance of polyacrylonitrile fibres to discolouration, comprising immers-

ing the never-dried fibres in an aqueous bath containing 0.5 percent to 2 percent of sodium formaldehyde bisulphite.

3. A process for increasing the resistance of polyacrylonitrile fibres to discoloration, comprising applying to the never-dried fibres, in an aqueous medium, a reducing agent selected from the group consisting of sodium metabisulphite, potassium metabisulphite, thiourea dioxide, formaldehyde, paraformaldehyde and addition

compounds with formaldehyde of a compound which has no adverse effect on the fibres.

4. A process according to claim 3, in which the aqueous medium contains 0.1 to 10 percent of the reducing agent.

5 **References Cited in the file of this patent**

**UNITED STATES PATENTS**

2,768,995 Mosse ----- Oct. 30, 1956